

# United States Patent

[11] 3,623,982

[72] Inventor **William Patrick Scott**  
**Ponca City, Okla.**  
[21] Appl. No. **729,425**  
[22] Filed **May 15, 1968**  
[45] Patented **Nov. 30, 1971**  
[73] Assignee **Continental Oil Company**  
**Ponca City, Okla.**

[54] **RUST-INHIBITED CALCIUM BASE GREASES**  
**8 Claims, No Drawings**  
[52] **U.S. Cl.** ..... **252/33.3,**  
252/34, 252/34.7, 252/36, 252/389, 252/392  
[51] **Int. Cl.** ..... **C10m 5/22,**  
C10m 5/20  
[50] **Field of Search** ..... **252/34,**  
34.7, 37, 36, 37.7, 51.5 A, 50, 33.3, 389, 33.6, 392

[56] **References Cited**  
**UNITED STATES PATENTS**  
2,858,273 10/1958 **Worth** ..... 252/36  
3,159,576 12/1964 **Cridle** ..... 252/51.5  
3,390,085 6/1968 **Floeck** ..... 252/34.7  
2,671,758 3/1954 **Vinograd et al.** ..... 252/33  
2,695,910 11/1954 **Asseff** ..... 252/33

*Primary Examiner*—Daniel E. Wyman

*Assistant Examiner*—I. Vaughn

*Attorneys*—Joseph C. Kotarski, Henry H. Huth, Jerry B. Peterson, Bayless E. Rutherford, Jr. and Carroll Palmer

**ABSTRACT:** This disclosure concerns calcium base greases containing a rust-inhibiting amount of a combination of lead naphthenate and didodecyl dimethyl quaternary ammonium nitrite (or nitrate). Preferably, the grease contains, also, a fatty imidazoline alkyl diamine dicaprylate. These greases are particularly suitable for use in salt-water environments.

## RUST-INHIBITED CALCIUM BASE GREASES

## BACKGROUND

Historically, calcium base greases were the first to be commercially produced in any volume. Over the years they have had the largest sale of any of the greases and continue to be popular. The reason for this large consumption is that they are economical, have good resistance to water, are stable at most temperatures ordinarily encountered and have a smooth texture.

Since calcium base greases have good resistance to water they are particularly suitable in marine applications. In the past it has been customary to incorporate a rust inhibitor in the grease to improve its resistance to corrosion. Most of the rust-inhibited greases of the prior art, including those which are commercially available, provide reasonably satisfactory service in fresh water. Unfortunately, in salt-water, or brackish water, the greases of the prior art are not too satisfactory. Accordingly, it is highly desirable to have a calcium base grease which provides outstanding rust inhibition in a salt-water environment.

It is an object of the present invention to provide such a grease.

## PRIOR ART

The use of lead naphthenate in greases is well known. For example, U.S. Pat. No. 3,355,384 teaches a lithium base grease containing a rust inhibiting amount of a combination of lead naphthenate and a petroleum oxidation product.

U.S. Pat. No. 3,159,564 teaches the use of quaternary ammonium compounds (e.g. dicocodimethyl ammonium chloride) to improve the yield of calcium base greases. This patent, however, contains not teachings that quaternary ammonium compounds are useful as a rust inhibitor.

To my knowledge there are no references which teach a grease composition containing a combination of lead naphthenate and didodecyl dimethyl ammonium nitrite, or of this combination containing, in addition, a fatty imidazoline alkyl diamine dicaprylate.

## BRIEF SUMMARY OF THE INVENTION

Broadly stated, my invention relates to calcium base greases containing a rust-inhibiting amount of a combination of lead naphthenate and dialkyl dimethyl quaternary ammonium nitrite (or nitrate).

In a preferred embodiment, my invention relates to calcium base greases containing a rust-inhibiting amount of a combination of lead naphthenate, dialkyl dimethyl quaternary ammonium nitrite (or nitrate) and a fatty imidazoline alkyl diamine dicaprylate.

Preferably, the dialkyl dimethyl quaternary ammonium nitrite is didodecyl dimethyl quaternary ammonium nitrite.

In one aspect, my invention relates to a method of lubricating machinery exposed to a salt-water environment wherein the lubricant is a calcium base grease containing a rust-inhibiting amount of a combination of lead naphthenate, dialkyl dimethyl quaternary ammonium nitrite (or nitrate) and a fatty imidazoline alkyl diamine dicaprylate.

## DETAILED DESCRIPTION

## Calcium Base Greases

Suitable calcium base greases for use in my invention include calcium soap greases and calcium sulfonate greases. The term "calcium soap" greases includes hydrate, anhydrous and complex greases. The book "Manufacture and Application of Lubricating Greases" by C. J. Boner (Reinhold Publishing Corp., pages 355-423 and Corp. New York, 1954) 640-649 describes calcium soap greases. In order to make my disclosure more complete these portions of the Boner book are made a part of this disclosure.

The calcium soap greases comprise a grease-forming amount of a calcium soap or calcium complex in a liquid

lubricating oil. The amount of calcium soap or calcium complex is suitably in the range of about 1 to about 25 percent by weight of the base grease. Preferably, the amount of calcium soap or calcium complex is in the range of about 5 to about 10 percent, by weight.

The liquid lubricating oil which is used in the calcium base greases of my invention can be either a mineral lubricating oil or a synthetic lubricating oil. Of these, the mineral lubricating oils are preferred. These can be derived from naphthenic or paraffinic base crude oils, and can be either residual or distillate oil or a mixture thereof, depending on the particular grease which is being prepared.

The term synthetic lubricating oil, as used herein, refers to materials derived synthetically which are suitable as lubricants. Examples of suitable synthetic lubricants include the silicones, polyalkylene glycols, fluorocarbons, esters of dicarboxylic acids, esters of long-chain carboxylic acids, and complex esters.

It is to be understood that the type of lubricating oil used in my greases is not critical, and that any of the lubricating oils which have heretofore been used to prepare calcium base greases are suitable.

The term "calcium sulfonate" grease refers to greases wherein the grease-forming agent is a calcium sulfonate. Preferably, the grease-forming agent is a hyperbasic calcium sulfonate. (The term "hyperbasic" means that the calcium sulfonate contains an excess of basic calcium compounds over that required to neutralize the sulfonic acid.)

An example of a suitable calcium sulfonate grease and a method of preparing same is taught by McMillen in U.S. Pat. NO. 3,242,079, which patent is made a part of this disclosure.

An alternative and particularly suitable process of preparing the calcium sulfonate grease is disclosed and claimed in application Ser. No. 727,719 filed May 8, 1968, and now abandoned which application is made a part of this disclosure.

It is to be understood that the present invention concerns only the rust-inhibited grease composition and not the process of preparing the calcium base grease.

40 The calcium sulfonate greases, preferably, have the following composition:

|                            | Suitable | Preferred |
|----------------------------|----------|-----------|
| 45 Nonvolatile diluent oil | 20-80    | 40-60     |
| Dispersing agent           | 5-55     | 15-30     |
| Basic calcium compound     | 1-45     | 3-35      |

These greases have a dropping point, ASTM, of at least 480° F. In addition they have an acetic base number of at least 50, preferably at least 135.

50 The terms "nonvolatile diluent oil" "dispersing agent" and "basic calcium compound" are described in the above-mentioned application. They are also described in U.S. No. 3,150,088, which patent is made a part of this disclosure.

55 Since the rust-inhibiting additive combination of my invention has been found to be suitable in several different types of calcium base greases, it is believed to be suitable for use in all calcium base greases.

## Rust-inhibiting Additive Combination

## Lead Naphthenate

The lead naphthenate which is used in the greases of my invention can be any commercially available lead naphthenate. A commercial grade of lead naphthenate containing about 30 percent, by weight, lead has been particularly suitable.

## 60 Quaternary Ammonium Nitrite (or Nitrate)

The dialkyl dimethyl quaternary ammonium nitrite or nitrate which is used in the greases of my invention can be represented by the following formula:



70 wherein X is nitrite or nitrate and R and R<sub>1</sub> are C<sub>9</sub> to C<sub>17</sub> groups. Preferably, R and R<sub>1</sub> are C<sub>12</sub> to C<sub>14</sub> alkyl groups and X



nary ammonium nitrite (Aquad 2C Nitrite) in varying amounts in the calcium sulfonate grease of example 1.

This example also illustrates the rust-inhibiting effect of a combination of lead naphthenate, didodecyl dimethyl quaternary ammonium nitrite (Aquad 2C Nitrite) and fatty imidazoline alkyl diamine dicaprylate (Nalco G39M), in varying amounts in the calcium sulfonate grease of example 1.

The modified ASTM test, using salt water, was employed. The results were as follows:

| WT. PERCENT IN BASE GREASE |                             |                                             |                                   |
|----------------------------|-----------------------------|---------------------------------------------|-----------------------------------|
| Lead naphthenate           | Quaternary ammonium nitrite | Fatty imidazoline alkyl diamine dicaprylate | Salt water rusting after one week |
| 2.0                        | 1.5                         |                                             | None to trace.                    |
| 2.0                        | 2.0                         |                                             | Trace.                            |
| 2.0                        | 3.0                         |                                             | Do.                               |
| 2.0                        | 4.0                         |                                             | Moderate.                         |
| 2.0                        | 1.5                         | 1.0                                         | None.                             |
| 2.0                        | 2.0                         | 1.0                                         | Do.                               |

#### EXAMPLE 4

This example provides comparative rust-inhibiting data on a number of commercially available greases, marketed for marine service.

The modified ASTM test, using salt water, was employed. The results were as follows:

| Grease | Grease-Forming Agent         | Salt water Rusting After One Week |
|--------|------------------------------|-----------------------------------|
| A      | Anhydrous Calcium Soap + ZnO | Severe rusting                    |
| B      | Calcium (Hydrated)           | Severe rusting                    |
| C      | Anhydrous Calcium            | Severe rusting                    |
| D      | Barium Soap + ZnO            | Severe rusting                    |
| E      | Calcium Complex              | Severe rusting                    |
| F      | Calcium Soap                 | Severe rusting                    |
| G      | Barium Soap                  | Severe rusting                    |

#### EXAMPLE 5

A. The base grease used in this example was a calcium sulfonate grease prepared in accordance with the procedure described and claimed in application Ser. No. 727,719. The specific procedure was as follows:

Charge:

328.1 g. Sulfonic acid  
82 g. 100 pale oil  
27.4 g. tap water

The above-listed materials were added to a 3-liter, 3-necked flask. An amount of 8.1 g. of  $\text{Ca}(\text{OH})_2$  was added for neutralization using methyl alcohol for addition. The contents of the flasks were mixed well for 5 minutes. Then the amount of  $\text{Ca}(\text{OH})_2$  for overbasing (67.5 g.) was added to the flask using methyl alcohol. A total amount of 174 g. of methyl alcohol was used.

The admixture was blown with  $\text{CO}_2$ , at a rate of about 4 g. per minute, for 20 minutes while maintaining the temperature at 35°-40° C. The contents were maintained at reflux temperature for 30 minutes. The contents of the flask were transferred to a Hobart mixer and heated at reflux temperature (115° F.) for 30 minutes. The admixture was then heated to 250° F. to remove solvents. A partial house vacuum was applied and the contents heated to a pot temperature of 325° F. The contents were cooled, 150 g. of bright stock (lubricating oil) was added, and then cooled to room temperature while mixing.

The yield of grease was 574 grams. The product had an ASTM penetration at 77° F. of 287.

B. Using the base grease described in part A of this example a grease was prepared having the following composition:

95.5% (wt.)

calcium sulfonate grease

75

|            |                                                             |
|------------|-------------------------------------------------------------|
| 2.0% (wt.) | lead naphthenate                                            |
| 1.5% (wt.) | didodecyl dimethyl quaternary ammonium nitrite <sup>1</sup> |
| 1.0% (wt.) | fatty imidazoline alkyl diamine dicaprylate <sup>2</sup>    |

5 <sup>1</sup>"Arquad" 2C NO<sub>2</sub>

<sup>2</sup>"Nalco" SCC 135

The compounded grease was tested using the modified ASTM method, employing lake water (Lake Ponca, Ponca City, Okla.). One of the better commercial greases was tested concurrently for comparative purposes. The results were as follows:

| 15 |                                     | Lake Water                       |                                   |                                     |
|----|-------------------------------------|----------------------------------|-----------------------------------|-------------------------------------|
|    |                                     | One Week<br>Roll-<br>Cone<br>ers | Two Weeks<br>Roll-<br>Cone<br>ers | Three Weeks<br>Roll-<br>Cone<br>ers |
| 20 | Commercial grease<br>Grease of this | M 8M<br>0 0                      | M 9M<br>0 0                       | S 11M<br>0 0                        |

The compounded grease was also tested using the modified ASTM method, employing Pacific Ocean water. The same commercial grease, as tested above, was also tested concurrently. The results were as follows:

| 30 |                                                           | Pacific Ocean Water              |                                   |                                     |
|----|-----------------------------------------------------------|----------------------------------|-----------------------------------|-------------------------------------|
|    |                                                           | One Week<br>Roll-<br>Cone<br>ers | Two Weeks<br>Roll-<br>Cone<br>ers | Three Weeks<br>Roll-<br>Cone<br>ers |
| 35 | Commercial grease<br>Grease of this<br>example<br>example | S 12S<br>T 4M<br>T 4M            | S 12S<br>T 2M<br>T 2M<br>10T      | S 12S<br>2M<br>M 2M<br>1T           |

40 In the two tables shown above the ratings had the following meaning:

0 = No corrosion

=T = Trace corrosion

M = Moderate corrosion

S = Severe rusting and metal penetration

45 There were 12 rollers for each bearing. The number preceding the rating indicates the number of individual rollers rusted. For example, 12S means that all rollers were rusted severely.

#### EXAMPLE 6

This example illustrates the effectiveness of the rust-inhibiting additive combination of my invention in a hydrated calcium grease.

55 A pressure type saponification vessel (1) was charged with the following materials to prepare concentrated soap stock:

158 pounds Distilled Tallow Fatty Acids (2)

23 pounds Calcium Hydroxide

6 pounds Water

60 325 pounds Oil (3)

The vessel was closed and the total mass was stirred and heated to about 350° F. During heating the vessel pressure increased to about 70 p.s.i. The result was a liquid soap which was removed from the saponification vessel into an open type grease kettle having counter-rotating scraper type agitators. Additional water was added while the hot soap stock was being agitated until at least 0.5 to 1.0 percent water could be maintained. Additional oil (488 pounds (4) was added slowly to the soap stock to make a finished base grease having a penetration of about 265 (5).

70 A composition containing the above grease was blended as follows:

573 parts above described grease

|          |                               |
|----------|-------------------------------|
| 12 parts | lead Naphthenate              |
| 9 parts  | didodecyl dimethyl quaternary |
|          | ammonium nitrite (Arquad      |
|          | 2C Nitrite)                   |
| 6 parts  | fatty imidazoline alkyl       |
|          | diamine dicaprylate (Nalco    |
|          | SCC 135)                      |

When tested in the modified ASTM D1743 rust test using Gulf ocean water, the bearing showed only trace rusting on one bearing after one week storage and no rusting after 2 weeks in storage.

1. Stratco contactor

2. Emery 531

3. A solvent neutral cycle oil having a viscosity of ~ 144 S.S.U. at 100° F. and ~ 42 S.S.U. at 210° F.

4. A solvent neutral cycle oil having a viscosity of ~ 900 S.S.U. at 100° F. and ~ 70 S.S.U. at 210° F.

5. ASTM D217 Method

#### EXAMPLE 7

This example illustrates the effectiveness of the rust-inhibiting additive combination of my invention in an anhydrous calcium grease.

The following materials were charged to a double planetary open-type grease kettle

3200 parts Paraffinic Oil (S.S.U. 80 at 100° F.)

108 parts Calcium Hydroxide

108 parts Water

700 parts 12-Hydroxystearic Acid

The above mixture was heated slowly (over a period of 2 hours) to 260° F. Additional oil was added slowly (2,000 parts S.S.U. 80 paraffinic oil). The total mass was then passed through a Charlotte Colloid mill set at 0.003-inch clearance.

A compounded grease composition was prepared by adding to the entire amount of the base grease the following materials:

|            |                               |
|------------|-------------------------------|
| 126 parts  | lead naphthenate              |
| 63 parts   | fatty imidazoline alkyl       |
|            | diamine dicaprylate (Nalco    |
|            | SCC 135)                      |
| 94.5 parts | didodecyl dimethyl quaternary |
|            | ammonium nitrite (Arquad      |
|            | 2C Nitrite)                   |

The resulting grease had a penetration of 275. When tested in the modified ASTM D1743 rust test using Gulf ocean water, the test bearings exhibited only trace to no corrosion.

#### EXAMPLE 8

This example illustrates the effectiveness of the rust-inhibiting additive combination of my invention in a calcium sulfonate - acetate complex grease.

The base grease was prepared by adding to an open-type planetary scraper-type grease vessel the following materials:

460 parts hyperbasic calcium sulfonate having an acetic base number of about 300

270 parts paraffinic bright stock oil (2,900 S.S.U. at 100° F. and 155 S.S.U. at 210° F.)

The above mixture was heated and stirred to 180° F. at which time 50 parts of water were added. The above mass was agitated for approximately 30 minutes while maintaining a temperature of between 210° and 220° F. A mixture of 45 parts of glacial acetic acid and 55 parts of water was then added slowly to the above mixture. The total mass was then agitated for about 30 minutes while maintaining a temperature of between 210° and 220° F. Water was then removed by heating the kettle contents to 310° F. at which time 270 parts of the above described oil were added. The resulting grease was cooled to 235° F. and the following materials added:

|          |                               |
|----------|-------------------------------|
| 21 parts | Lead Naphthenate              |
| 16 parts | didodecyl dimethyl quaternary |

|          |                            |
|----------|----------------------------|
| 11 parts | ammonium nitrite (Arquad   |
|          | 2C Nitrite)                |
|          | fatty imidazoline alkyl    |
|          | diamine dicaprylate (Nalco |
|          | SCC 135)                   |

The resulting grease had a penetration of 267.

When tested in the modified ASTM D1743 rust test, using Gulf ocean water, the test bearings exhibited a trace to moderate corrosion.

#### EXAMPLE 9

This example illustrates the effectiveness of the rust-inhibiting additive combination of my invention in a calcium sulfonate-acetate-fatty acid complex grease.

The base grease was prepared by adding to an open-type planetary scraper-type grease vessel the following materials:

|    |            |                              |
|----|------------|------------------------------|
| 20 | 249 parts  | hyperbasic calcium sulfonate |
|    |            | having an acetic base        |
|    | 96 parts   | number of about 300          |
| 25 | 1.25 parts | paraffinic Bright stock oil  |
|    | 25 parts   | (same as in example 8)       |
|    |            | methoxy ethanol              |
|    |            | water                        |

The above mixture was stirred for 30 minutes while maintaining a temperature of 210° to 220° F. 5.45 parts of 12-hydroxystearic acid were added followed by a mixture of 24.3 parts glacial acetic acid and 30 parts water. This mixture was stirred for 30 minutes while maintaining a temperature of 210° to 220° F. The total mass was then heated to 310° F. to remove water and the following added:

|    |            |                               |
|----|------------|-------------------------------|
| 35 | 97 parts   | paraffinic Bright Stock oil   |
|    | 43 parts   | paraffinic Pale Oil (S.S.U.   |
|    |            | 100 at 100° F.)               |
| 40 | 12.9 parts | Lead Naphthenate              |
|    | 9.7 parts  | didodecyl dimethyl quaternary |
|    |            | ammonium nitrite (Arquad      |
|    | 6.5 parts  | 2C Nitrite)                   |
|    |            | Fatty imidazoline alkyl       |
|    |            | diamine dicaprylate (Nalco    |
|    |            | SCC 135)                      |

45 The resulting grease had a penetration of 271.

When tested in the modified ASTM D-1743 rust test, using Gulf ocean water, the test bearings exhibited only a trace to no corrosion.

50 The rust-inhibiting additive composition of my invention has not been found to be effective in preventing salt water corrosion when added to lithium-base greases. For this reason it is believed that the additive composition is specific for calcium greases.

55 It is to be understood that various other additives which are normally used in greases can be used in my greases. Examples of these additives include oxidation inhibitors, lubricating agents, extreme pressure agents, stringiness agents and the like.

60 While particular embodiments of the invention have been described, it will be understood, of course, that the invention is not limited thereto, since many modifications may be made; and it is, therefore, contemplated to cover by the appended claims any such modifications as fall within the true spirit and scope of the invention.

65 The invention having been described, what is claimed and desired to be secured by Letters Patent is:

70 1. A grease composition consisting essentially of a calcium base grease, made with a mineral lubricating oil, containing synergistic rust-inhibiting proportions of a combination of lead naphthenate, a fatty imidazoline alkyl diamine dicaprylate prepared from a fatty imidazoline alkyl diamine having the structure



wherein R is mixed heptadecenyl or mixed heptadecadienyl, and a dialkyl dimethyl quaternary ammonium compound represented by the formula



wherein R and R<sub>1</sub> are C<sub>9</sub> to C<sub>17</sub> alkyl groups and X is nitrite or nitrate.

2. The grease composition of claim 1 wherein the lead naphthenate is present in an amount of from about 1 to 3 percent by weight, the fatty imidazoline alkyl diamine dicaprylate is present in an amount of from about 0.5 to about 2 percent by weight and the dialkyl dimethyl quaternary ammonium compound is present in an amount of from about 1 to about 4 percent by weight.

3. The grease composition of claim 2 wherein the base grease is a calcium sulfonate grease.

4. The grease composition of claim 2 wherein the base grease is a calcium soap grease.

5. A grease composition consisting essentially of a calcium base grease, made with a mineral lubricating oil, containing synergistic rust-inhibiting proportions of a combination of lead naphthenate, a fatty imidazoline alkyl diamine dicapry-

5

late prepared from a fatty imidazoline alkyl diamine having the structure



10

wherein R is mixed heptadecenyl or mixed heptadecadienyl, and a dialkyl dimethyl quaternary ammonium compound represented by the formula



20

where R and R<sub>1</sub> are C<sub>9</sub> to C<sub>17</sub> alkyl groups and X is nitrite or nitrate, said lead naphthenate being present in an amount of from about 1.5 to about 2.5 percent by weight, said fatty imidazoline alkyl diamine dicaprylate being present in an amount of from about 0.75 to about 1.25 percent by weight and said dialkyl dimethyl quaternary ammonium compound being present in an amount from about 1.25 to about 2 percent by weight.

6. The grease composition of claim 5 wherein the quaternary ammonium compound is didodecyl dimethyl quaternary ammonium nitrite.

7. The grease composition of claim 6 wherein the base grease is a calcium sulfonate grease.

8. The grease composition of claim 6 wherein the base grease is a calcium soap grease.

35

\* \* \* \* \*

40

45

50

55

60

65

70

75